

# UNITED STATES PATENT OFFICE.

WILHELM HELMUTH SCHWEITZER, OF HEIDELBERG, GERMANY, ASSIGNOR TO SOCIETY "TECHNOCHEMIA" AKTIENGESELLSCHAFT, OF GLARUS, SWITZERLAND.

## TEXTILE PRODUCT DERIVED FROM ANIMAL FIBER AND A PROCESS OF MAKING SAME.

1,389,274.

Specification of Letters Patent. Patented Aug. 30, 1921.

No Drawing.

Application filed April 28, 1921. Serial No. 465,288.

To all whom it may concern:

Be it known that I, WILHELM HELMUTH SCHWEITZER, a citizen of the German Republic, and resident of Heidelberg, Germany, have invented a new and useful Textile Product Derived from Animal Fibers and a Process of Making Same, (for which I have filed an application in Germany, January 21, 1919,) of which the following is a full, clear, and exact specification.

For more than 20 years wool fiber has been treated with chlorin in order to prevent its felting and its shrinking or shortening when treated with hot liquids, to insure its easy dying in printing and to give it a silky appearance.

It is known that instead of chlorin other oxidizing chemicals have been employed.

There have been for a short time only yarns for knitting on the market, which had been treated with chlorin or bromin. But owing to their hard and dry feel and owing to the loss of their luster by washing, these yarns disappeared quickly from the market.

On the other hand, wool fiber has already been produced which had, it is true to say, the appearance and the feel of ordinary wool fiber and did not shorten or shrink, when washed in a hot bath.

When treating wool fiber with chlorin, hydrochloric acid is produced and, of course, little quantities of this acid, which may have remained in the fiber, have always been neutralized with some alkali.

Nevertheless for this purpose only very little quantities of alkali were necessary and only in great dilution and there never existed any intention to produce any reaction

between the alkali and the very substance of the chlorinated wool fiber, probably while any reaction has always been carefully avoided in order to not spoil the strength and the other good properties of the wool fiber.

Now I have found the surprising fact, that wool fibers previously treated with chlorin or any other oxidizing chemicals as well as hairs and all other known animal textile fibers previously chlorinated can be transformed into fibers of an entirely new kind, which complete most fortunately the assortment at the disposal of the spinner.

The remarkably increased luster, strength,

soft feel and elasticity of the so transformed fibers will insure them a large employment.

The means used for producing this curious transformation, which is especially valuable for hairs which heretofore have been of much less value than the wool fiber itself, may be described as follows:

Animal fiber of any sort and in any condition, as flocks, slivers, yarn or cloth, is treated with chlorin or other oxidizing agents in a known manner. Thereby these oxidizing agents can be employed in excess in view of obtaining the maximum of the oxidizing effect.

The oxidized fiber, which contrary to the non-treated wool fiber, which is an amino-acid, is probably a polyoxyaminoacid, is then dipped into a bath containing relatively high quantities of alkali, as for instance soda lye or sodium carbonate, in respect to the weight of the fiber.

A violent reaction takes place between the alkali and the oxidized fiber, the bath becomes colored and the oxidized fiber becomes transparent, slippery and at the same time very brilliant.

The slippery consistence disappears more and more by rinsing the treated fiber and by treating it with boiling soap solutions (this treatment is advantageously preceded by a drying process) and the new fiber acquires its characteristic properties which are a high luster, an increased strength and increased elasticity, and a remarkably soft and silky feel, especially when care has been taken to give a finish at ordinary temperature with a little acetic acid or to calender after drying.

Accordingly to the desired effect and the concentration of the alkaline baths employed the transformation of the fiber occurs at a higher or a lower temperature and in the course of a longer or a shorter time.

The use of an excess of alkali is one of the most characteristic features of the invention.

In the above given example the wool fiber, previously treated for example with chlorin, is dipped for a rather short time into a bath which contains as much of soda lye (caustic soda) as would correspond to 30 per cent. of the weight of the wool fiber. Instead of pure alkali, I may also use al-

kaline baths containing compounds of alkali with certain organic substances, as for example phenols, or soaps or other substances softening the action of the caustic alkali such as for instance molasses, glucose, glycerin, etc.

The fiber previously treated with an oxidizing agent and an excess of alkali can be impregnated subsequently with a water-proofing and softening substance, as for instance, wax, paraffin, stearin, resins, vegetable wax, either by passing the fiber through a bath of these bodies in a melted state and removing afterward the excess of the same by pressure, or by solvents or boiling soap baths, or by passing the fiber through a solution of the said bodies or a solution of the said bodies previously saponified. If the said bodies employed are previously saponified an excess of alkali may remain in the soap solution and act thus on the chlorinated or otherwise treated fiber.

The fiber treated with an oxidizing agent can also be at first impregnated with the water-proofing and softening substance and treated subsequently with the alkaline bath in order to remove the excess of the water-proofing and softening substance from the surface of the fiber. In all cases sufficient of the water-proofing substance remains in the fiber for obtaining the desired effect.

If the water-proofing and softening substance, as such or previously saponified, be employed in the form of a solution, the treatment with the alkaline bath precedes advantageously the treatment with the said solution of water-proofing and softening substance, in order to avoid that the water-proofing and softening substance deposited in the fiber be removed again therefrom.

*Example.*

50 kilos of a fine wool cloth are treated at ordinary temperature with a filtered solution of 40 kilos of chlorid of lime in 1500 liters of water to which an equivalent quantity of hydrochloric acid has been previously added, until the developed hypochlorous acid disappears, which is generally the case after half an hour. The cloth is then abundantly rinsed with cold water. Afterward it is bleached by dipping it into a solution of sodium hydrosulfite or of sulfurous acid and rinsed. Then the bleached fiber is boiled in a solution of 3 kilos of wax soap in 1500 liters water and rinsed in cold water. (The wax soap employed is prepared by saponifying 3 parts of bee's wax with 3 parts of solid soda lye). The cloth is then treated for a relatively short time, varying from a few minutes to  $\frac{1}{4}$  of an hour, according to the thickness of the fiber or other reasons, with a solution of 15 kilos of solid soda lye in 1500 liters of water, wrung out and again copiously rinsed with water. Finally the cloth

is boiled in a solution of Marseille soap to which at the end some acetic acid has been added, dried and calendered.

What I claim is:

1. As a new article of manufacture, the herein described textile product derived from an animal fiber, which results from the successive treatment of an animal fiber with an oxidizing agent and an excess of alkali and shows a higher luster, a higher strength and a higher elasticity than the animal fiber from which it is derived and a remarkably soft and silky feel and is also more transparent than the animal fiber from which it is derived. 80

2. As a new article of manufacture, the herein described textile product derived from an animal fiber, which results from a successive treatment of an animal fiber with an oxidizing agent and an excess of alkali, is impregnated with a water-proofing and softening substance and shows a higher luster, a higher strength and a higher elasticity than the animal fiber from which it is derived and a remarkably soft and silky feel 90 and is also more transparent than the animal fiber from which it is derived. 90

3. The herein described process for the manufacture of a textile product derived from an animal fiber, consisting in treating an animal fiber first with an oxidizing agent and afterward with an excess of alkali. 95

4. The herein described process for the manufacture of a textile product derived from an animal fiber, consisting in treating an animal fiber successively with an oxidizing agent and an excess of alkali and impregnating the fiber finally with a water-proofing and softening substance. 100

5. The herein described process for the manufacture of a textile product derived from an animal fiber, consisting in treating an animal fiber successively with an oxidizing agent, an excess of alkali and a solution of a water-proofing and softening substance. 110

6. The herein described process for the manufacture of a textile product derived from an animal fiber, consisting in treating an animal fiber first with an oxidizing agent, then impregnating the fiber with a water-proofing and softening substance and finally treating it with an excess of alkali. 115

7. The herein described process for the manufacture of a textile product, derived from an animal fiber, consisting in treating an animal fiber successively with an oxidizing agent, a solution of a water-proofing and softening substance and an excess of alkali. 120

8. The herein described process for the manufacture of a textile product derived from an animal fiber, consisting in treating an animal fiber successively with an oxidizing agent, a bleaching agent, a solution of a water-proofing and softening substance and an excess of alkali. 125 130

9. The herein described process for the manufacture of a textile product derived from an animal fiber, consisting in treating an animal fiber successively with an oxidizing agent and an excess of a solution of alkali containing a substance capable of softening the action of the alkali.

10. The herein described process for the manufacture of textile product from an animal fiber, consisting in treating successively the fiber with an oxidizing agent and an excess of alkali, impregnating the fiber with

a water-proofing and softening substance and finally treating the fiber with a boiling soap bath, in order to remove the water-proofing and softening substance from the surface of the fiber. 15

In witness whereof I have hereunto signed my name this 30th day of March, 1921, in the presence of two subscribing witnesses.

**WILHELM HELMUTH SCHWEITZER.**

Witnesses:

EMILE BRONNERT,  
AMAND GRANN.